

Patented May 10, 1927.

1,628,160

# UNITED STATES PATENT OFFICE.

MORRIS CHARLES LAMB, OF BERMONDSEY, LONDON, ENGLAND.

## PREPARATION AND DYEING OF LEATHER.

No Drawing. Application filed June 9, 1925, Serial No. 36,052, and in Great Britain April 27, 1925.

This invention relates to the dyeing of leather and provides a treatment which effects the equal distribution and solubilization of the natural grease in the skins and 5 enables them to be dyed a level shade of color and also gives greater penetration of the dyestuff and enhancement of the color produced.

According to this invention I treat the 10 leather with a solution or emulsion of a compound containing a naphthalene nucleus. The term is used in the generally accepted sense as representing a nucleus of the form

15



containing from 8 to 16 hydrogen atoms. The leather employed may be tanned either 20 by vegetable or mineral tanning agents or dressed by the oil or aldehyde process. It has been found that the treatment by the compound containing the naphthalene nucleus applied either before or during the 25 process of dyeing effects solubilization of the natural and artificial grease contained in the leather and the leather is so modified that the dyestuff penetrates more deeply than is usually the case and there is considerable 30 increase in the intensity of shade produced. Various compounds of the type referred to can be used but the compound preferred is 35 hydrogenated naphthalene, used either alone in a soluble or finely divisible form or in an emulsified form obtained by the employment of emulsifying agents, e. g. sodium, potassium or ammonium ricinoleate, hydrogenated phenol soaps, hydrogenated cresol soaps, sulphonated or soluble oils of vegetable, animal, 40 or mineral origin, the salts of sulphonated aromatic acids, or aromatic acids either used alone or in conjunction with each other; or the employment of a mixture of an emulsion or solution of hydrogenated naphthalene in 45 conjunction with halogen or other hydrocarbon compounds.

The method of treatment may be considerably varied and the following are four examples of the treatment, out of many which 50 could be employed:—

### Example 1.

Vegetable tanned leathers, such as basils,

East India tanned sheepskins and hides, 55 bark and sumach tanned calfskins, skivers, roans, etc., are first treated with water either cold or warm in a drum, paddle or other vessel for any desired period until thoroughly wetted, when for each 100 lbs. leather, 1 to 60 3 lbs. of a 90 per cent emulsion of hydrogenated naphthalene is added, and the goods treated in the mixture for a period of about 15 minutes, when the requisite coal-tar dye-stuff is then added and the treatment con- 65 tinued for a further period of 45 minutes.

### Example 2.

Vegetable tanned leathers, such as enumerated above, are first thoroughly wetted 70 out, when an addition is made to the vessel of 2 per cent to 3 per cent of a 90 per cent emulsion of hydrogenated naphthalene, and the goods processed for any desirable period. They are then washed and dyed with coal- 75 tar or natural dyestuffs by any of the common methods in use.

### Example 3.

Chrome tanned leather, after being washed and the acidity neutralized in the ordinary manner, is transferred to a suitable vessel and treated with 3 per cent to 5 per cent of a 90 per cent emulsion of naphthalene in conjunction with sodium ricinoleate and tri-chlorethylene, for a period of about half-an-hour. The requisite dyestuff for dyeing the leather is then added and the dyeing process proceeded with in the ordinary way. 80 85 90

### Example 4.

Vegetable, mineral tanned, or oil dressed or aldehyde leather is first wetted in water by any of the ordinary methods and is then 95 treated with 2 per cent to 3 per cent of an emulsion of 70 per cent hydrogenated naphthalene, 10 per cent hydrogenated phenol soap, and 10 per cent ordinary ammonia or potash soap, for a period of 30 minutes, 100 when the dyeing process is proceeded with, either by the addition of the requisite coal-tar or natural dyestuff to the solution, or by separate treatment by any ordinary method.

It is to be understood that the term emulsion as used in the claims is intended to cover also a solution of the naphthalene compound in cases where a solution is feasible. 105

What I claim and desire to secure by Letters Patent of the United States is:—

1. In the dyeing of leather, treating the leather with an emulsion of hydrogenated naphthalene and with a dyeing agent.
2. In the dyeing of leather, a process which consists in adding an emulsion of hydrogenated naphthalene to the dye bath.
3. In the dyeing of leather, a process which consists in employing an emulsion of a compound containing a naphthalene nu-

cleus in conjunction with coal-tar colouring matter and with a halogen hydrocarbon.

4. In the dyeing of leather, treating the leather with an emulsion of a compound containing a naphthalene nucleus together with a soluble ricinoleate.

5. A process as in claim 4, in which trichlorethylene is also employed with the aforesaid substances.

MORRIS CHARLES LAMB.